

July 19, 1932.

F. C. SCHLUDECKER

1,867,767

TWO-TONE ORNAMENTATION OF STAINLESS IRON

Filed Aug. 21, 1931

Fig. 1.



Fig. 2.



Fig. 3.



Fig. 4.



Inventor

Fred C. Schludecker

By *Clarence O'Brien*  
Attorney

## UNITED STATES PATENT OFFICE

FRED C. SCHLUDECKER, OF MASSILLON, OHIO

## TWO-TONE ORNAMENTATION OF STAINLESS IRON

Application filed August 21, 1931. Serial No. 558,613.

This invention relates to the method of and means for producing ornamentation of stainless iron, the general object of the invention being to provide means for covering certain portions of the stainless metal and then treating the other portion to produce designs, lettering or the like so as to produce an attractive two tone finish similar to etching but more economically produced.

10 This invention also consists in certain other features of construction and in the combination and arrangement of the several parts to be hereinafter fully described, illustrated in the accompanying drawing and 15 specifically pointed out in the appended claim.

In describing the invention in detail, reference will be had to the accompanying drawing wherein like characters denote like or corresponding parts throughout the several views, and in which:

Figure 1 is a view of the stainless metal with the stencil sheet thereon.

25 Figure 2 is an edge view of Figure 1.

Figure 3 is an edge view showing the covering medium in place on the plate.

Figure 4 is a view of the completed plate.

In these views the letter A indicates the plate of stainless metal, and the letter B the

30 stencil plate attached to one face thereof.

The parts of the plate exposed by the stencil are treated with varnish, after which the varnish is baked at a temperature of preferably 250° F. Of course, the parts which are not 35 to be treated may be covered with other material such as fiber paper.

The stencil B is then removed and the exposed portion not covered by the varnish or fiber paper or other material is covered with 40 a composition preferably consisting of powdered pumice, oil, lime, and kerosene after which the exposed parts are worked with a tantico brush or buff thereby producing a beautiful two-tone finish similar to etching but more economically produced.

The above mentioned ingredients are used in approximately the following proportions:—4 parts kerosene, 1 part engine oil, 3 parts powdered pumice, 1 part burnt lime.

45 By this method any letters, design, land-

scape, or other ornamental work now done by the etching process can be produced and it will have as much or more beauty.

This invention can be used for producing name-plates, signs, grave markers, lettering 55 of all kinds, etc.

Figure 3 shows the sheet after the varnish or other covering material is applied as shown at 1 and Figure 4 shows the polished or not treated surfaces of the plate at 2 and 60 the treated portions at 3.

It is thought from the foregoing description that the advantages and novel features of the invention will be readily apparent.

It is to be understood that changes may be 65 made in the construction and in the combination and arrangement of the several parts provided that such changes fall within the scope of the appended claim.

## I claim:

The herein described method of producing designs, letters, etc., on stainless metal consisting in covering certain portions of the metal with a protective covering and then 75 treating the other portions with a composition composed of powdered pumice, oil, lime and kerosene and working the surface so covered with the composition with a brush or buff.

70 In testimony whereof I affix my signature.

FRED C. SCHLUDECKER.

65

70

75

80

85

90

95

100